

# United States Patent

[11] 3,617,335

[72] Inventors **Shiro Kimura;**  
Teruo Kobayashi; Sadao Ishige, all of  
Kanagawa, Japan

[21] Appl. No. 842,008

[22] Filed July 15, 1969

[45] Patented Nov. 2, 1971

[73] Assignee Fuji Photo Film Co., Ltd.  
Kanagawa, Japan

[32] Priority July 15, 1968

[33] Japan

[31] 43/49817

Primary Examiner—Murray Katz  
Attorney—Sughrue, Rothwell, Mion, Zinn & Macpeak

**ABSTRACT:** A pressure-sensitive copying paper comprising a support having coated thereon microcapsules containing an organic solvent solution of a compound which, when in contact with an electron acceptable solid acid, forms a color dye and is represented by the following formula:



[54] **PRESSURE-SENSITIVE COPYING PAPER**  
5 Claims, No Drawings

[52] U.S. Cl. .... 117/36.2,  
117/36.9, 260/310

[51] Int. Cl. .... B41m 5/22

[50] Field of Search .... 117/36.2,  
36.8, 36.9; 260/310 R

[56] **References Cited**  
UNITED STATES PATENTS

|           |        |              |       |            |
|-----------|--------|--------------|-------|------------|
| 3,491,116 | 1/1970 | Lin          | ..... | 260/326.14 |
| 3,499,902 | 3/1970 | Coles et al. | ..... | 260/287    |
| 3,509,174 | 4/1970 | Lin          | ..... | 260/326.14 |

wherein R<sub>1</sub> and R<sub>2</sub> each represents a member selected from the group consisting of an alkyl group having from one to five carbon atoms and a benzyl group; X represents a member selected from the group consisting of an alkyl group having from one to five carbon atoms and an aryl group, and Y represents a member selected from the group consisting of an alkyl group having from one to 17 carbon atoms, an aryl group, an amino group, an acylamino group and an alkoxy group having from one to five carbon atoms.

1  
PRESSURE-SENSITIVE COPYING PAPER

## BACKGROUND OF THE INVENTION

## 1. Field of the Invention

This invention relates to a pressure-sensitive copying paper and in particular, it is concerned with a pressure-sensitive copying paper using as a color former a compound represented by the following general formula:



in which  $R_1$  and  $R_2$  are alkyl groups of one to five carbon atoms or benzyl groups,  $X$  is an alkyl group of one to five carbon atoms or an aryl group, and  $Y$  is an alkyl group of one to 17 carbon atoms, an aryl group, an amino group, an acylamino group or an alkoxy group.

## 2. Description of the Prior Art

Ordinary pressure-sensitive copying paper consists of an upper paper onto which is coated a substantially colorless organic compound having an electron-donating property and a color forming reactivity (hereinafter referred to as a "color former") dissolved in an organic solvent and incorporated in microcapsules and a lower paper, onto which is coated electron-acceptable solid acid. If necessary, an intermediate paper layer is provided onto one side thereof is coated the color-former-containing microcapsules and on the other side thereof is coated a solid acid, and a support on one side of which the microcapsules and solid acid are coated.

In the case of using the upper and lower paper in combination with the optional intermediate paper, the papers are pressed locally in such a manner that the microcapsules-containing layer and the solid acid-containing layer are contacted, whereby the microcapsules in this pressurized area are broken and the color former is reacted with the solid acid, thus color forming.

In the case of using a pressure-sensitive copying paper having the microcapsules and solid acid on the same side, the paper may be pressed for color forming by means of a typewriter, for example.

Examples of color formers coloring in red and blue are the following: leuco triphenylmethane derivatives, leuco methylene blue acyl derivatives, and triphenylmethane and xanthene phthalide derivatives having lactone rings. However, there are not many color formers coloring in yellow orange to orange red. These color formers have the following disadvantages. That is to say, o-hydroxybenzalacetophenone has a low color forming density. 2-(4-hydroxystyryl)-3,3-dimethyl-3H-indole or 2-(4-acetamidestryl)-3,3-dimethyl-3H-indole (cf. Japan Pat. publication No. 21033/1966) has a high color forming density and relatively strong light resistance after color forming, but the light resistance before color forming and water resistance after color forming are weak. If a color former coloring in yellow-orange to orange-red is obtained which has a higher color density, higher color forming speed and stronger light resistance and water resistance before and after color forming than those known in the art, a pressure-sensitive copying paper coloring in yellow-orange to orange-red as well as a pressure-sensitive copying paper coloring in an optional color such as black or blue-black used together with a known color former coloring in red or blue will be given. This advantage enlarges the application of pressure-sensitive copying papers.

## SUMMARY OF THE INVENTION

It is the principal object of the present invention to obtain a pressure-sensitive copying paper coloring in yellow-orange to orange-red as well as to provide a pressure-sensitive copying paper coloring in an optional color such as black or blue-black together with a known red or blue color former by the use of a compound represented by the foregoing general formula.

We have discovered as a result of many studies on a color former coloring in yellow-orange to orange-red that the use of a compound represented by the foregoing general formula as a color former leads to obtaining a pressure-sensitive copying paper coloring in yellow-orange to orange-red as well as a pressure-sensitive copying paper coloring in an optional color such as black or blue-black when used together with a known color former coloring in red or blue.

## DETAILED DESCRIPTION OF THE INVENTION

20 A pressure-sensitive copying paper according to the present invention using the compound of the foregoing general formula has an excellent stability in air before color forming, is free from coloring and lowering of the color forming ability, colored in yellow-orange to orange-red immediately when contacted with an electron-accepting solid acid, thus resulting in a high color density and is strongly resistant to light and water after color forming. When used together with a known color former coloring in red or blue, it colors in various colors such as black and blue-black without being desensitized.

25 30 Typical examples of the compound coloring in yellow-orange to orange-red, represented by the foregoing general formula, are as follows;

(1)



(2)



(3)





60 The aryl groups of X and Y in the foregoing general formula can be nonsubstituted phenyl groups, nonsubstituted naphthyl groups, and phenyl groups and naphthyl groups substituted with groups such as alkyl groups, halogen atoms, alkoxy groups, acetoxy groups, acylamino groups, acyl groups and nitro groups, excluding those groups which liberate ions such as sulfonic groups, carboxyl groups, and hydroxyl groups.

65 The compound represented by the foregoing general formula is prepared by the following procedure. 2-(4'-dialkylamino-2'-hydroxybenzoyl) benzoic acid is reacted with the corresponding pyrazolone in concentrated sulfuric acid at a reaction temperature of 30°-100° C. for 3-24 hours. The reaction solution is then cooled to room temperature and poured into a large amount of ice water and the precipitated product is filtered and then treated with an aqueous alkaline solution to thus obtain a colorless crystal.



Identification of the thus obtained compound with the molecular structure of the general formula is carried out by IR absorption spectrum and elementary analysis. The characteristic absorption of carbonyl in the lactone ring of these compounds appears near 1,755 cm.<sup>-1</sup> and neither the characteristic absorption of other carbonyl groups, except in the foregoing color former (9) having a carbonyl of amide, nor the characteristic absorption of a hydroxyl group was found. The result of the elementary analysis corresponds to the theoretical value as shown in the following synthesis examples.

The typical electron-accepting solid acids used in the invention are active clay materials such as acid clay, active clay, attapulgite, zeolite and bentonite, and solid organic acids such as succinic acid, tannic acid, gallic acid and pentachlorophenol.

As the organic solvent for dissolving the color former, the following may be used: ethylene glycol, chlorobenzene and chlorinated diphenyl.

The typical preparation methods of the compound represented by the foregoing general formula are illustrated by the following synthesis examples:

#### SYNTHESIS EXAMPLE 1

Preparation of the color former (1) represented by the general formula wherein



14.3 g. of 2-(4'-dimethylamino-2'-hydroxybenzoyl) benzoic acid (1/20 mol) and 8.7 g. of 3-methyl-1-phenylpyrazolone (1/20 mol) were dissolved in 72 g. of concentrated sulfuric acid (94-96 percent) at below 45°C., reacted at 90°±2°C. for 3 hours, and cooled to room temperature. The reaction solution was then poured into 800 g. of ice water, followed by filtering. The precipitate was extracted with 600 ml. of chloroform while being neutralized with an aqueous solution of caustic soda. The chloroform solution was washed with water several times and concentrated under reduced pressure to obtain 14.6 g. of a colorless crystal melting at 296°-298°C.

Analysis of the crystal:

Found (percent by weight): C, 73.41; H, 4.93; N, 9.80.  
Calculated for  $C_{26}H_{21}N_{3}O_3$ : C, 73.74; H, 5.00; N, 9.92.

#### SYNTHESIS EXAMPLE 2

Preparation of the color former (2) represented by the general formula wherein



15.7 g. (1/20 mol) of 2-(4'-diethylamino-2'-hydroxybenzoyl) benzoic acid and 8.7 g. (1/20 mol) of 3-methyl-1-phenylpyrazolone were reacted and processed in a similar manner as in Synthesis Example 1 to thus obtain 19.5 g. of a colorless crystal melting at 260°-261°C.

Analysis of the crystal:

Found (percent by weight): C, 74.23; H, 5.57; N, 9.37.  
Calculated for  $C_{28}H_{25}N_3O_3$ : C, 74.48; H, 5.58; N, 9.31.

#### SYNTHESIS EXAMPLE 3

Preparation of the color former (3) represented by the general formula wherein

General Formula

10



15 18.8 g. (1/20 mol) of 2-(4'-benzylethylamino-2'-hydroxybenzoyl) benzoic acid and 8.7 g. (1/20 mol) of 3-methyl-1-phenylpyrazolone were reacted and processed in a similar manner as in Synthesis Example 1 to thus obtain 21.4 g. of a colorless crystal melting at 198°-202°C.

Analysis of the crystal:

Found (percent by weight): C, 77.21; H, 5.18; N, 8.64.  
Calculated for  $C_{32}H_{25}N_3O_3$ : C, 76.93; H, 5.04; N, 8.41.

#### SYNTHESIS EXAMPLE 4

Preparation of the color former (4) represented by the general formula wherein



15.7 g. (1/20 mol) of 2-(4'-diethylamino-2'-hydroxybenzoyl) benzoic acid and 9.4 g. (1/20 mol) of 3-methyl-1-(p-tolyl)-(p-tolyl) pyrazolone were reacted and processed in a similar manner as in Synthesis Example 1 to thus obtain 21.0 g. of a colorless crystal melting at 186°-187°C.

Analysis of the crystal:

Found (percent by weight): C, 74.68; H, 5.78; N, 9.10.  
Calculated for  $C_{29}H_{27}N_3O_3$ : C, 74.82; H, 5.85; N, 9.03.

#### SYNTHESIS EXAMPLE 5

Preparation of the color former (5) represented by the general formula wherein



15.7 g. (1/20 mol) of 2-(4'-diethylamino-(2'-hydroxybenzoyl) benzoic acid and 13.9 g. (1/20 mol) of 3-methyl-1-(2',4',6'-trichlorophenyl) pyrazolone were reacted and processed in a similar manner as in Synthesis Example 1 to thus obtain 23.2 g. of a colorless crystal melting at 213°-214°C.

Analysis of the crystal:

Found (percent by weight): C, 60.70; H, 4.06; N, 7.68; Cl, 18.98.

Calculated for  $C_{26}H_{22}Cl_3N_3O_3$ : C, 60.61; H, 4.00; N, 7.57; Cl, 19.17.

#### SYNTHESIS EXAMPLE 6

Preparation of the color former (6) represented by the general formula wherein



15.7 g. (1/20 mol) of 2-(4'-diethylamino-2'-hydroxybenzoyl) benzoic acid and 15.4 g. (1/20 mol) of 3-ethoxy-1-(2',4',6'-trichlorophenyl) pyrazolone were dissolved in 72 g. of concentrated sulfuric acid (94-96 percent) at below 40°C,

reacted at 50° C. for 6 hours and at 60° C. for 3 hours and processed in a similar manner in Synthesis Example 1 thus to obtain 21.7 g. of a colorless crystal melting at 178°-180° C.

Analysis of the crystal:

Found (percent by weight): C, 59.48; H, 4.06; N, 7.26; Cl, 18.07.

Calculated for  $C_{29}H_{24}Cl_1N_3O_4$ : C, 59.55; H, 4.13; N, 7.18; Cl, 18.18.

#### SYNTHESIS EXAMPLE 7

Preparation of the color former (7) represented by the general formula wherein



15.7 g. (1/20 mol) of 2-(4'-diethylamino-2'-hydroxybenzoyl) benzoic acid and 11.8 g. (1/20 mol) of 1,3-diphenyl-pyrazolone were reacted and processed in a similar manner as in Synthesis Example 1 to thus obtain 20.8 g. of a colorless crystal melting at 205° C.

Analysis of the crystal:

Found (percent by weight): C, 77.14; H, 5.26; N, 8.27. Calculated for  $C_{33}H_{27}N_3O_3$ : C, 77.17; H, 5.30; N, 8.18

#### SYNTHESIS EXAMPLE 8

Preparation of the color former (8) represented by the general formula wherein



15.7 g. (1/20 mol) of 2-(4'-diethylamino-2'-hydroxybenzoyl) benzoic acid and 8.7 g. (1/20 mol) of 3-amino-1-phenyl-pyrazolone were dissolved in 60 g. of concentrated sulfuric acid at below 40° C., reacted at 50° C. for 12 hours and at 60° C. for 3 hours and processed in a similar manner as in Synthesis Example 1 to thus obtain 18.6 g. of a colorless crystal melting at 265°-267° C.

Analysis of the crystal:

Found (percent by weight): C, 71.48; H, 5.40; N, 12.47. Calculated for  $C_{27}H_{24}N_4O_3$ : C, 71.66; H, 5.35; N, 12.38.

#### SYNTHESIS EXAMPLE 9

Preparation of the color former (9) represented by the general formula wherein



15.7 g. (1/20 mol) of 2-(4'-diethylamino-2'-hydroxybenzoyl) benzoic acid and 15.6 g. (1/20 mol) of 3-(p-chlorobenzoyl) amino-1-phenylpyrazolone were dissolved in 72 g. of concentrated sulfuric acid at below 40° C., reacted at 50° C. for 18 hours, neutralized with an aqueous solution of sodium carbonate at below 5° C. extracted with chloroform and the concentrated under reduced pressure to thus obtain 23.6 g. of a colorless crystal melting at 246°-226° C.

Analysis of the crystal:

Found (percent by weight): C, 68.88; H, 4.49; N, 9.63; Cl, 5.89.

Calculated for  $C_{34}H_{27}Cl_1N_4O_4$ : C, 69.09; H, 4.60; N, 9.48; Cl, 6.00.

Calculated for  $C_{34}H_{27}Cl_1N_4O_4$ : C, 69.09; H, 4.60; N, 9.48; Cl, 6.00.

#### SYNTHESIS EXAMPLE 10

Preparation of the color former (10) represented by the general formula wherein  $R_1=R_2=Et$ , and  $X=Y=Me$ .

15.7 g. (1/20 mol) of 2-(4'-diethylamino-2'-hydroxybenzoyl) benzoic acid and 5.6 g. (1/20 mol) of 1,3-dimethyl-

pyrazolone were reacted and processed in a similar manner as in Synthesis Example 9 followed by crystallizing from a mixed solvent of benzene-ether to thus obtain 15.3 g. of a colorless crystal melting at 177°-178° C.

Analysis of the crystal:

Found (percent by weight): C, 70.81; H, 6.01; N, 10.77.

Calculated for  $C_{23}H_{23}N_3O_3$ : C, 70.92; H, 5.95; N, 10.79.

#### SYNTHESIS EXAMPLE 11

Preparation of the color former (11) represented by the general formula wherein



15.7 g. (1/20 mol) of 2-(4'-diethylamino-2'-hydroxybenzoyl) benzoic acid and 38.4 g. (1/20 mol) of 3-heptadecyl-1(p-phenoxyphenyl)pyrazolone were reacted and processed in a similar manner as in Synthesis Example 9 to obtain a colorless syrupy material. The spectra of this material exhibited an absorption band at  $\lambda_{max}=505.485$  millimicrons in 95 percent acetic acid solution.

Analysis of product:

25 Found (percent by weight): C, 78.06; H, 7.89; N, 5.41. Calculated for  $C_{50}H_{46}N_3O_4$ : C, 78.24; H, 7.95; N, 5.48.

For the production of the pressure-sensitive copying paper of the present invention using the compound represented by the general formula, a method of making microcapsules by 30 utilizing the complexed coacervation is employed, for example, which is disclosed in U.S. Pat. Nos. 2,548,366, 2,800,457 and 2,800,458 as being well-known to those skilled in the art. The instant invention is characterized by the use of the compound represented by the foregoing general formula as a color former. The characteristics of the pressure-sensitive copying paper are independent from the production method thereof. The amount of the color former used is generally 0.5-5 percent by weight based on the organic solvent.

40 The following examples are given in order to further illustrate the pressure-sensitive copying paper of the present invention using the typical color formers represented by the general formula, the examples being nonlimiting in nature.

#### EXAMPLE 1

Three grams of each of the color formers (1)-(11) was taken and processed according to the following procedure. The color former was dissolved in 100 g. of trichlorodiphenyl. To the resulting solution were added 20 g. of gum arabic and 50 160 g. of water at 50° C. to give an emulsion, further, 20 g. of acid-treated gelatin and 160 g. of water and then acetic acid were added, while stirring to adjust the pH to 5. Then, 500 g. of water was added thereto to advance the coacervation to 55 form a thickened liquid film of gelatin-gum arabic around the oil drop of trichlorodiphenyl dissolving the color former. After adjusting the pH to 4.4, 3.8 g. of a 37 percent aqueous solution of formalin was added thereto to harden the liquid film, and then an aqueous caustic soda solution was added to adjust the 60 pH to 9 while being cooled to 10° C. and the resulting mixture was allowed to stand for 5-6 hours to complete the coacervation. The thus capsulized liquid was coated onto a sheet of paper by roll coating or by air knife coating and then dried. When the coated paper (upper paper) was brought into close 65 contact with another sheet of paper (lower paper) coated with an electron-accepting solid acid such as acid clay, active clay, attapulgite, zeolite or bentonite and pressed by means of a pencil or typewriter, there instantaneously occurred a thick color formation on the pressed area of the lower sheet of 70 paper. The color varied with the variety of the color formers although it was independent of the variety of the above-mentioned clays. A yellow-orange color was noted in the color formers (1), (2), (4), (5), (6) and (10) orange in (3), (7), and (11); and orange-red in (8) and (9). These color formed dyes were scarcely faded even though exposed to direct sunlight for

a long time or wetted with water. Moreover, a similar color formation was given thereto even when using a lower sheet of paper coated with an organic solid acid such as succinic acid, gallic acid, p-toluenesulfonic acid, pentachlorophenol or phenol resin. No lowering of the color forming ability in the color former coated paper (upper paper) was found even though heated at 100° C. for 20 hours or exposed to the sunlight for a long time.

#### EXAMPLE 2

The procedure of example 1 was repeated, except that 1.51 g. of the color former (2) was used with the known color formers, i.e., 0.3 g. of Benzoyl Leuco Methylene blue, 0.5 g. of Malachite Green Lactone, 0.7 g. of Crystal Violet Lactone, 0.3 g. of N-phenyl-leuco auramine and 0.4 g. of Rhodamine B Anilinolactam. When the thus-coated paper (upper paper) was brought into close contact with a paper (lower paper) coated with an electron-accepting solid acid, and then pressed, there rapidly occurred a color formation of black on the lower sheet of paper.

#### EXAMPLE 3

The procedure of example 1 was repeated, except that 0.3 g. of the color former (4) and 0.7 g. of the color former (8) 25 were used with 0.5 g. of Benzoyl Leuco Methylene Blue, 2.0 g. of Crystal Violet Lactone and 0.8 g. of N-phenyl-leuco auramine. When the thus-obtained pressure-sensitive copying paper was pressed by writing, there rapidly occurred a color formation of blue-black.

#### EXAMPLE 4

The procedure of example 1 was repeated, except that 1.8 g. of the color former (7) was used with 1.2 g. of Rhodamine B Anilinolactam. The thus-obtained pressure-sensitive copying paper was colored in bright red. When using Rhodamine B Anilinolactam alone, the color was bluish red that felt too dark to be used practically.

#### EXAMPLE 5

The procedure of example 1 was repeated, except that the capsule was applied to a lower sheet of paper coated with a clay in place of using two sheets of paper. Pressing of the superposedly coated paper gave the same color formation as in example 1.

What is claimed is:

1. A pressure-sensitive copying paper comprising a support having coated thereon microcapsules containing an organic solvent solution of a compound which, when in contact with an electron acceptable solid acid, forms a color dye and is represented by the following formula:



wherein R<sub>1</sub> and R<sub>2</sub> each represents a member selected from the group consisting of an alkyl group having from one to five carbon atoms and a benzyl group; X represents a member selected from the group consisting of an alkyl group having

from one to five carbon atoms and an aryl group, and Y represents a member selected from the group consisting of an alkyl group having from one to 17 carbon atoms, an aryl group, an amino group, an acylamino group and an alkoxy group having from one to five carbon atoms.

2. The pressure-sensitive copying paper as in claim 1 wherein said organic solvent is a member selected from the group consisting of chlorinated diphenyl, chlorobenzene and ethyleneglycol.

10 3. The pressure-sensitive copying paper as claimed in claim 1 wherein said electron-acceptable soil acid is a member selected from the group consisting of an acid clay, an active clay, attapulgite, zeolite, bentonite, succinic acid, tannic acid, gallic acid and pentachlorophenol.

15 4. A pressure-sensitive copying paper comprising a support having coated thereon an electron-acceptable solid acid and microcapsules containing an organic solvent solution of a compound which is in contact with said electron-acceptable solid acid to form a color dye and is represented by the following formula:



30

wherein R<sub>1</sub> and R<sub>2</sub> each represents a member selected from the group consisting of an alkyl group having from one to five carbon atoms and a benzyl group, X represents a member selected from the group consisting of an alkyl group having from one to five carbon atoms and an aryl group, and Y represents a member selected from the group consisting of an alkyl group having from one to 17 carbon atoms, an aryl group, an amino group, an acylamino group and an alkoxy group having from one to five carbon atoms.

35 5. A pressure-sensitive copying paper comprising and under paper having coated thereon an electron-acceptable solid acid and an upper paper having coated thereon microcapsules containing an organic solvent solution of a compound which is in contact with said electron-acceptable solid acid to form a color dye and is represented by the following formula:



40

55 60 wherein R<sub>1</sub> and R<sub>2</sub> each represents a member selected from the group consisting of an alkyl group having from one to five carbon atoms and a benzyl group, X represents a member selected from the group consisting of an alkyl group having from one to five carbon atoms and an aryl group, and Y represents a member selected from the group consisting of an alkyl group having from one to 17 carbon atoms, an aryl group, an amino group, an acylamino group and an alkoxy group having from one to five carbon atoms.

\* \* \* \* \*

UNITED STATES PATENT OFFICE  
CERTIFICATE OF CORRECTION

Patent No. 3,617,335 Dated November 2, 1971

Inventor(s) Shiro Kimura et al.

It is certified that error appears in the above-identified patent and that said Letters Patent are hereby corrected as shown below:

Column 1, line 34, after "coated" insert -- an --; line 36, after "provided" insert -- and --. Column 5, line 38, "and Y = Me" should read -- and Y = Me. --; line 60, "and Y = Me" should read -- and Y = Me. --. Column 7, line 2, "thus to" should read -- to thus --. Column 8, line 30, after "coacervation" insert -- technique --; line 31, "which is" should read -- that --; same line 31, "patent" should read -- Patent --. Column 9, line 44, "i" should read -- in --. Column 10, lines 44 and 45, "which is in contact" should read -- which, when contacted --; line 45, "acid to form" should read -- acid, forms --.

Signed and sealed this 13th day of June 1972.

(SEAL)

Attest:

EDWARD M. FLETCHER, JR.  
Attesting Officer

ROBERT GOTTSCHALK  
Commissioner of Patents